

July 14, 1936.

S. P. MILLER

2,047,742

SIDING ELEMENT AND PROCESS OF MAKING SAME

Filed June 14, 1933



INVENTOR

Stuart P. Miller

BY *Forbes Shelly*

ATTORNEY

## UNITED STATES PATENT OFFICE

2,047,742

SIDING ELEMENT AND PROCESS OF  
MAKING SAMEStuart Parmelee Miller, Englewood, N. J., assignor  
to The Barrett Company, New York, N. Y., a  
corporation of New Jersey

Application June 14, 1933, Serial No. 675,777

11 Claims.

(Cl. 91—68)

This invention is directed to siding elements and more particularly to siding elements of the felt base type coated with waterproofing material and surfaced with granular material. The 5 term "siding elements" is used in a broad sense and is intended to include shingles or other elements applied to a roof as well as elements applied to a wall.

One object of the invention is to provide a durable and weather resistant light weight siding element which can readily be applied to walls or other surfaces. The invention comprehends a ready and efficient procedure for making such siding elements as well as the elements themselves.

Another object of this invention is to provide weather resistant and light weight siding elements in which carbonaceous material, such as ground coke, is used for surfacing the top and/or the under side of a coated base, thus resulting in a lighter and more durable element as compared with the well known mineral surfaced elements.

Other objects and advantages will appear from the following detailed description of my invention.

It has been proposed to manufacture felt base siding elements by coating both sides of a bitumen-saturated felt base with bituminous coating material, such as asphalt, partially embedding mineral grit, such as crushed slate, in the coating 20 on both sides of the element, and thereafter applying a second coating of bituminous material and a second surfacing of mineral grit on that portion of the element adapted to be exposed to the weather.

In accordance with a preferred form of my invention carbonaceous surfacing material may be employed for covering the seal-back coating on the under side of the element and for surfacing both coatings on the side of the element exposed to the weather when laid. By the term "carbonaceous surfacing materials" is meant ground petroleum coke, ground pitch coke, ground coal coke, bone charcoal, vegetable carbon, or similar material.

The siding of my invention possesses important advantages over sidings heretofore known and used. As compared with mineral granules now employed, carbonaceous surfacing material, such as ground coke, used in accordance with my invention, is more durable and less susceptible to weather influences such as deterioration. Accordingly, the siding elements of my invention are much more weather resistant than elements heretofore made and provide a more durable and lasting structure. Furthermore, the bituminous

coating material in which the coke particles are embedded tends to enter the numerous pores and crevices in the carbonaceous particles and become firmly bonded therewith. Hence a lasting bond between the bituminous coating layer and the carbonaceous surfacing material results.

A substantial economy is effected by the use of carbonaceous material, such as ground coke, since it is considerably cheaper than the mineral grit heretofore used. Furthermore, carbonaceous 10 material such as ground coke is considerably lighter in weight than mineral granules and results in economies in the shipping, handling, and application of the elements.

For a better understanding of the invention 15 reference should be made to the accompanying drawing wherein is shown by way of illustration a preferred embodiment of the invention and in which:

Fig. 1 is a side elevation, somewhat diagrammatic in character, and shows the steps involved in the manufacture of the siding elements of this invention;

Fig. 2 is a fragmentary plan view of the first 20 coating and surfacing apparatus, a portion of the sheet being shown in plan for the sake of clearness;

Fig. 3 is a fragmentary plan view of the second coating and surfacing apparatus showing a portion of the coated and surfaced sheet;

Fig. 4 is a fragmentary plan view of a finished 25 coated and surfaced sheet and indicates the layout for cutting the sheet into individual elements;

Fig. 5 is a plan view of a siding element and 30 illustrates a preferred embodiment of this invention;

Fig. 6 is a vertical section taken along the line 35 6—6 of the siding element of Fig. 5; and

Fig. 7 is a fragmentary plan view of a number 40 of overlapping courses, each composed of siding elements of this invention laid in abutting relationship.

Referring to the drawing, with particular reference to Fig. 1, a sheet of fibrous material 1, which may be and preferably is of the usual roofing felt 45 made of rag fiber, paper stock, or other fibrous material, with or without suitable fillers as well known in this art, is fed by feed rolls 2 from the usual paper making machine or felt roll into a looping device 3. From the looping device 3, rolls 4 feed the sheet into any suitable type of saturating apparatus, indicated generally by the reference numeral 5. Saturating tank 6 may contain suitable cementitious waterproofing composition, such as asphalt or other bituminous material, 55

utilized for the impregnation and saturation of roofing felts.

Rolls 7 and 8 feed the saturated sheet to a second looping device 9. The passage of the saturated fibrous sheet or base through the looping device 9 gives the saturant an opportunity to dry and to thoroughly impregnate the base. Rolls 11 and 12 feed the saturated sheet from the looping device 9 to the coating appliance indicated 10 generally by the reference numeral 13 having a pair of coating rolls 14 and 15. Feed rolls 12 are preferably driven at substantially the same average peripheral speed as the coating rolls 14 and 15. A sufficient amount of slack should be provided and maintained between the driven rolls 12 and guide rolls 16 over which the sheet passes before entering the bite of the coating rolls 14 and 15 to prevent tearing of the sheet if the rate of rotation of coating rolls 14 and 15 should momentarily increase relatively to the rate of rotation of rolls 12. Coating roll 15 is rotatably mounted in a tank 17 which may contain bituminous material, such as asphalt or other cementitious waterproofing substance, suitable for coating roofing felt.

As the sheet 1 passes between coating rolls 14 and 15, the under side of the sheet is completely coated by roll 15. Waterproofing material is applied to the top of the sheet before passing 30 through the coating rolls by means of a supply pipe 18 equipped with a discharge spout 19 of a width approximately equal to that of the sheet, as shown in Fig. 2. The coating material is spread uniformly over the top and bottom surfaces of the sheet as it passes between the coating rolls 14 and 15 in the form of a top coating layer 20 and a rear or seal-back coating.

Immediately after leaving the coating appliance 13 and while the coating material is still soft and 40 tacky, the coated sheet passes under a surfacing device or hopper 22 extending across the width of the sheet. Carbonaceous material, such as ground coke, is fed into this hopper and is showered by means of the usual distributing roll 23 45 onto the coated base passing thereunder covering substantially the entire surface of the sheet with surfacing material.

After being surfaced, the sheet passes about 50 reversing roll 25 which functions to partially embed the ground coke in the tacky and plastic coating. Any excess coke granules fall from the surfaced sheet into hopper 22 from whence they were showered onto the coated sheet.

In the continued passage of the surfaced sheet, 55 it travels next under hopper 26. Finely divided carbonaceous material such as ground or powdered coke of a size corresponding to that of sand is deposited in hopper 26 and is discharged therefrom by distributing roll 27 onto the seal-back 60 coating in the form of a surfacing layer covering substantially the entire under side of the sheet. The sheet then passes over reversing roll 28 which partially embeds the powdered coke in the seal-back coating and imparts a relatively smooth 65 surface to the back of the sheet. Excess carbonaceous material falls from the sheet as the latter passes from reversing roll 28 over a series of calender rolls 30 where the product is given an opportunity to cool.

From the calendar rolls 30 the sheet now having 70 a single coating and single surfacing of carbonaceous material on both the top and under sides, is passed between coating rolls 31 and 32 of the second coating device indicated in general by 75 reference numeral 33. Upper coating roll 31 is

composed of three sections as shown in Fig. 3 each of a width equal to approximately twice the width of that portion of the finished siding element adapted to be exposed to the weather when laid. Waterproofing material from any suitable 5 source is applied to the top of the sheet by means of feed pipes 34 equipped with discharge spouts 35. As shown in Fig. 3, these feed pipes and spouts are preferably three in number and are positioned over the sheet so as to feed the waterproofing material onto the sheet directly in front of each section of the coating roll 31. The coating material discharged from the spouts is spread uniformly over the surfaced sheet in the form of coating lanes 36 as the sheet passes between the 15 coating rolls.

Immediately after leaving the second coating appliance, and while the second coating is still soft and tacky, the sheet passes under a second surfacing device 38. As shown in Figs. 1 and 3, 20 this device consists of three hoppers 39 each adapted to hold carbonaceous surfacing material and each equipped with a distributing roll 40. Granular carbonaceous material, such as ground coke, preferably of a different size from the granules fed from hopper 22, is deposited in these hoppers. The material is showered by means of the distributing rolls onto the lanes of coating material and adheres thereto forming surfaced bands 41. The thus surfaced sheet then passes 30 about reversing roll 42 which functions to partially embed the granules in the lanes 36 of plastic coating material. Any granules which may fall on the previously surfaced areas or bands 43 adjacent and between lanes 36 do not adhere 35 thereto. When the sheet leaves reversing roll 42 such granules and the excess granules on the surfaced bands 41 fall therefrom back into the hoppers 39.

The double coated and double surfaced sheet 40 next passes over a reversing roll 44 to the drying and pressing rolls 45. Feed rolls 46 feed the sheet from the pressing rolls into a looping device 47 where the product is given an opportunity to cool. From the looping device 47 the surfaced sheet 45 passes through rolls 48 to cutting cylinders 50. These cylinders simultaneously cut rows of slots 51 in the double coated and surfaced portions of the sheet as shown in Fig. 4. The individual slots of each row are of a length preferably equal to the width of the double-surfaced bands 41. The sheet is simultaneously cut longitudinally along longitudinal lines 52 intersecting the slots 51 midway between the ends thereof and also along lines 53 coinciding with the median lines of the single surfaced areas 43. Simultaneously with the longitudinal cutting operations the base is cut transversely along lines indicated by the reference numeral 54.

The transverse cuts 54 are spaced apart a distance corresponding to the length of the desired elements and are of such a shape, as shown in Fig. 4, that one transverse edge of each element is formed with a triangular projection while the other transverse edge is provided with a complementary recess. Preferably the slotting and longitudinal and transverse cutting operations are accomplished by passing the surfaced sheet through cutting rolls which substantially simultaneously make all the cuts. The cutting operations, however, may be carried out in any desired order, the slotting operation preceding or following the cutting of the base into longitudinal strips. From the cutting cylinders 50 the cut sheet passes through knocker and ejector cylin- 70 75 80 85 90 95

ders 56 of any well known type which remove any portions of the material cut out to form the slots which may adhere to the cut sheets. From the tab ejector mechanism the individual siding elements pass to suitable stacking appliance (not shown).

The siding resulting from the above described operations is shown in Figs. 5 and 6. That portion of each element adapted to be exposed to the weather when laid is provided with a series of cut outs or slots 57 defining a plurality of rectangular shaped tabs 58. Side edge 59 is formed with a triangular projection 60 and the other side edge 61 has a complementary triangular recess 62. Each element consists of a felt base 63 having a seal-back coating 64 of bituminous water-proofing composition, such as asphalt, rendered non-cementitious by the application thereto of an overlying layer 65 of powdered or ground carbonaceous material, such as ground coke. The top side of the element is substantially completely covered by coating layer 67 having a surfacing layer 68 of carbonaceous material partially embedded therein. The surfacing layer 25 covers both the tabs and the body portion of the element. A second coating 69 of waterproofing composition overlies the surfacing on the tabs and has a surfacing layer 70 of carbonaceous material partially embedded in its surface.

30 The element of Figs. 5 and 6 is designed to be laid in overlapping courses with the triangular projection 60 snugly fitting within the recess 62 of a contiguous element in the same course as shown in the top course of Fig. 7. Hence, the triangular projection and complementary triangular recess aid in aligning the elements in each course. The elements are preferably so laid that the forward edges of the elements of one course lie a short distance above the upper edges of the 40 double-surfaced tabs of the elements in the next underlying course. The resultant arrangement of the elements presents an appearance of a brick wall as shown in Fig. 7.

It will be noted that the siding element of this 45 invention involves substantially no waste in its manufacture, can be readily applied even by unskilled workmen, and when applied in the intended manner presents a wall having a regular and pleasing appearance. The use of carbonaceous surfacing material, such as ground coke, results in an improved siding element which is exceedingly durable and weather resistant since I have found that carbonaceous material is highly resistant to water, snow, and other weathering influences. The carbonaceous granules become firmly embedded in and attached to the coating material and do not become loosened in handling and after application. In addition they bond with the coating layers. Moreover, since 50 carbonaceous material, such as ground coke, costs less than mineral grit, the siding of this invention is more economical to manufacture than the mineral-surfaced siding elements heretofore commonly employed. In addition the elements of this 55 invention are lighter in weight than those heretofore produced and, consequently, are more readily handled, shipped, and applied.

In connection with the foregoing description and illustration of the preferred siding of this 60 invention and the method of making this siding, it should be understood that these are merely for the purpose of clarifying an understanding thereof. Various changes and modifications may be made within the scope of this invention.

75 Although carbonaceous material is preferably

exclusively used in the surfacing operations, talc may be used in surfacing the coating on the under side of the elements and carbonaceous material used only in surfacing the top coating layers. Conversely, the carbonaceous material may 5 be applied to the seal-back coating to render it non-cementitious and the coating layers on the face of the elements surfaced with mineral grit.

Since certain other changes in carrying out the process and in the constructions set forth may be 10 made without departing from the scope of this invention, it is intended that all matter contained in the above description or shown in the accompanying drawing shall be interpreted as 15 illustrative and not in a limiting sense. 15

I claim:

1. The process of making siding elements which comprises coating a felt base with cementitious waterproofing material, surfacing the waterproofing material with finely divided carbonaceous material, applying cementitious waterproofing material in selected areas over the carbonaceous material on the top side of the base, partially embedding finely divided carbonaceous material in the last mentioned waterproofing material, and cutting the base into siding elements. 25

2. The process of making siding elements which comprises coating both sides of a felt base with cementitious waterproofing material, surfacing both sides of the base by partially embedding 30 ground coke in the waterproofing material, applying spaced lanes of cementitious waterproofing material on the top side of the surfaced base, partially embedding ground coke in said lanes, and cutting the resultant base into siding elements. 35

3. The process of making siding elements having rectangular tabs along one longitudinal edge thereof which comprises coating both sides of a felt base with bituminous material, surfacing both sides of the coated base with ground coke, 40 applying spaced longitudinal lanes of bituminous material over the ground coke on the top side of the base, surfacing said lanes with ground coke, cutting rows of spaced slots through the surfaced lanes, and cutting transversely through the single 45 coated and single surfaced areas between the lanes and longitudinally along lines intersecting the rows of slots to form said elements.

4. A siding element comprising a fibrous base, cementitious waterproofing material covering the 50 weather and under sides of the base, layers of carbonaceous material partially embedded in the waterproofing material, a coating of waterproofing material covering portions of the carbonaceous material on the top side of the base, 55 and a layer of carbonaceous material partially embedded in said coating.

5. A siding element comprising a fibrous base having tabs along one longitudinal edge of the body portion thereof, the top and under sides of 60 said base being covered with cementitious waterproofing material, carbonaceous material partially embedded in the waterproofing material on both sides of the base, a layer of cementitious waterproofing material overlying the surfacing 65 material on the top side of the tabs, and carbonaceous material partially embedded in said layer of waterproofing material.

6. A siding element comprising a felt base having both sides covered with bituminous material, ground coke partially embedded in the bituminous material on both sides of the base, a layer of bituminous material overlying the coke on the exposed portions of the base, and ground 75

coke partially embedded in said last mentioned bituminous material.

- 5 7. A siding element adapted to be laid with other like elements in overlapping courses, the elements of each course being in abutting relationship, comprising a felt base coated on both sides with bituminous material and having tabs along one longitudinal edge thereof, said tabs being separated by slots, carbonaceous surfacing 10 material partially embedded in the bituminous material on both sides of the element, bituminous material covering the carbonaceous surfacing material on the tab portions of the element, and carbonaceous surfacing material partially embedded in said bituminous material, the slots between the tabs extending up from the lower edge of the element to a depth coextensive with the double-coated and double-surfaced portions of the element.
- 15 8. The process of making siding elements which comprises coating a base with a layer of cementitious waterproofing material and surfacing the layer of waterproofing material with a layer of ground granular carbonaceous material, the waterproofing material entering the pores and crevices of said carbonaceous material so that the surfacing layer adheres firmly to the coating 20 layer.
- 25

9. The process of making siding elements which comprises coating the top side of a fibrous base with a layer of cementitious waterproofing material, applying a layer of ground granular coke and partially embedding it in said layer of cementitious waterproofing material, said waterproofing material entering the pores and crevices of said coke to bond the latter firmly to said coating layer.

10. A siding element comprising a base coated with a layer of cementitious waterproofing material and surfaced with a layer of ground carbonaceous material partially embedded in the layer of waterproofing material, said waterproofing material entering the pores and crevices of said carbonaceous material whereby firm adhesion of the carbonaceous material to the waterproofing material is secured.

11. A siding element comprising a felt base provided with a seal-back coating of cementitious waterproofing material, a layer of ground coke partially embedded in said coating, said coating material entering the pores and crevices of said ground coke whereby to unite the latter firmly with said layer of waterproofing material.

STUART PARMELEE MILLER.